

# UNITED STATES PATENT OFFICE.

GILBERT RIGG, OF MELBOURNE, VICTORIA, AUSTRALIA, ASSIGNOR TO MINING AND METALLURGICAL PROCESSES PROPRIETARY LIMITED, OF MELBOURNE, VICTORIA, AUSTRALIA.

## DESULFURIZATION OF ZINC SULFID ORES.

1,401,733.

Specification of Letters Patent. Patented Dec. 27, 1921.

No Drawing.

Application filed May 21, 1918. Serial No. 235,784.

To all whom it may concern:

Be it known that I, GILBERT RIGG, metallurgist, a subject of the King of Great Britain, residing at Melbourne, in the State of 5 Victoria, Commonwealth of Australia, have invented certain new and useful Improvements in the Desulfurization of Zinc Sulfid Ores, of which the following is a specification.

10 This invention relates to certain improvements in the desulfurizing of zinc sulfid ores and refers more especially to the desulfurizing of blende concentrates (both granular material and slimes) preparatory to the 15 recovery of metallic zinc or spelter therefrom by distillation or leaching for electro-deposition or the production of zinc oxid.

Hitherto the desulfurization of zinc sulfids has been effected by roasting in rever- 20 beratory or muffle furnaces with more or less continuous rabbling either by hand or mechanical means for the purpose of maintaining the ore particles as far as possible in contact with the oxidizing atmosphere and 25 for the elimination of sulfur dioxid gases occluded in the ore.

In order to effectively desulfurize zinc sulfid ores it has been found necessary hitherto to first crush the ore to such a size as 30 will pass through from 8 to 20 mesh, per linear inch according to the character of the ore.

When the ore to be treated has been previously concentrated, as for instance by 35 gravity or flotation, it is usually in a still finer state of division. This fine condition of the ore while necessary for the roasting has serious drawbacks when the ore is submitted to reduction and distillation in re- 40 torts. In the first place it interferes seriously with the transmission of heat from the walls of the retorts to the body of the charge while further there is a greater tendency to fuse with the formation of slag. As 45 is well known in retort practice it is desirable to eliminate slagging as far as possible both on account of the destructive effect of the slag upon the retorts and also on account of the difficulty of drawing partly slagged 50 residues from the retorts. Again the fineness of the charge retards the reduction of the metal within the retorts by hindering the free circulation of carbon monoxid gas formed within the retorts which, as it comes 55 into contact with the particles of zinc oxid

reduces them to metal. Similarly the reduction of carbon dioxid gas, formed during the foregoing reaction is hindered. Numerous attempts have been made to devise means for providing charges of roasted or desulfurized zinc blende of coarser grain, but so far such results have not been satisfactory for many reasons.

In the first place it has been found impossible to roast or desulfurize zinc sulfid ores 60 such as zinc blende in coarse pieces. Such pieces with a diameter of approximately one quarter of an inch when submitted to a roasting or desulfurizing operation have been found to have an outer coating of zinc 65 oxid with a substantial kernel or core of unaltered sulfid. Such partially roasted ore has been found to give very poor results in the retort with in many cases a highly de- 70 structive action on the clays of which the re- 75 torts are composed. Furthermore zinc blende which has been submitted to a previous treatment by gravity concentration or flotation usually comes to the smelter in a much finer state of subdivision.

Attempts have been made to briquet the ore with coal or other carbonaceous fuel before charging the same into the retorts but such briquetting operations have not up to the present been successful. If the bri- 85 quets are sufficiently compressed to insure them not crumbling in the retorts they are too compact to enable them to work quickly, while if they crumble the advantage of bri- 90 queting is nullified.

Blende ores have not hitherto been amenable to blast roasting—that is by causing a current of air to pass through a body or bed of the ore which was previously ignited—owing to the excessive heat generated caus- 95 ing fusion and preventing contact between the ore particles and the oxidizing atmosphere.

The object of this invention is to provide certain improvements in the desulfurizing 100 of zinc sulfid ores whereby the elimination of the sulfur may be effected more economically and effectively than heretofore yielding a product of roasted or desulfurized ore in coarse grained form in lumps of a porous 105 nature and in a form suitable for reduction in distillation retorts and for leaching for electro-deposition and the production of zinc oxid.

I accomplish this object by effecting the 110

desulfurizing of blende ores in two separate operations the first of which comprises a partial roast for the dilution of the sulfur contents and the second of which consists 5 of subjecting the said partially roasted ore to a blast roasting operation that is to say igniting the charge and causing a current of air or oxidizing atmosphere to pass through the ore whereby the combustion of 10 the sulfur is maintained and the ore finally desulfurized and a product obtained in the form of a sinter.

In carrying out this invention any form 15 of "blast roaster" may be employed in which a current of air or oxidizing atmosphere is drawn or forced through a bed or charge of ore but the apparatus which I have found effective is the well known "Dwight and Lloyd" machine in which the 20 ore is delivered on to the surface of traveling grates which pass beneath an ignition burner after which the said grates travel over a suction chamber whereby air is drawn through the bed of ore. It will, however, be 25 understood that the purpose of the invention may be effected by employing other forms of blast roasters in which a current of air or oxidizing atmosphere is blown or drawn through a charge or bed of ore on a per- 30 forated grate and it will be understood that in this specification the term "Blast roaster" or its equivalent will include all such types of apparatus.

For the purpose of this invention it is 35 essential that the sulfur contents of the ore should be reduced in the first operation to such an extent that the heat generated in the second or blast roasting operation will not be sufficient to cause fusing or slagging. 40 Such reduction of the sulfur contents may be effected in several ways, such as,

(1) By partially roasting the ore until the sulfur contents are reduced to say from 8 to 10% and then subjecting the said par- 45 tially roasted ore to blast roasting.

(2) By partially roasting a certain por- 50 tion of the ore and mixing such partially roasted ore with green or unroasted ore in such proportions that the mixture has a sulfur content of say 8 to 10% and then sub- 55 jecting such mixture to blast roasting.

(3) By more or less completely roasting or desulfurizing the ore (such as to a dead roast) and mixing such desulfurized ore 55 with green or unroasted ore in such proportions that the mixture has a sulfur content of say from 8% to 10% and then subjecting such mixture to blast roasting.

In some cases I may effect the purpose of 60 this invention by subjecting the ore to a preliminary roast in a reverberatory or muffle or other suitable furnace for the elimination of part of the sulfur and subjecting such partially roasted ores to "blast roast- 65 ing" in which air or oxidizing atmosphere

is drawn or forced through the charge. In the working of such a method the most economical arrangement would be to work each type of roaster between its most effective limits and for this purpose I prefer to use a 70 multiple hearth roaster and conduct the operations therein so that the ore is reduced down to about 8 to 10% sulfur. Reducing the ore to about 8 to 10% sulfur is, however, merely illustrative, as the actual percent- 75 age is dependent on the particular ore treated, the invention residing rather in the result than in the actual percentage of sulfur removed. This partially roasted ore with or without damping as may be necessary is 80 then fed on to the grate of a "blast roaster" the desulfurized ore being in the form of a sinter suitable for subsequent treatment for the recovery of the zinc or the production of zinc oxid.

In many cases after a preliminary roast in the reverberatory furnace or muffle furnace as above indicated it is found that the ore contains a certain proportion of grains which have an external coating of zinc oxid 90 surrounding the internal kernel or core of unaltered sulfid. This condition tends to interfere with the rapid ignition of the charge in the blast roaster. I have found that this condition may be overcome by adding to the 95 ore coming from the aforesaid preliminary roast or desulfurization a small proportion of unroasted or green sulfids. This un- 100 roasted ore not having any inert coating rapidly ignites and helps to bring up the temperature to a point at which roasting and sintering of the ore proceeds at a satisfactory rate.

In practice the proportion or quantity of 105 roasted ore to the green sulfids is estimated according to the amount required to avoid fusing of the ore particles in the subsequent treatment.

For example in the treatment of Broken Hill zinc sulfid ores it has been found that 110 an ore roasted to 8% sulfur in a preliminary desulfurization when mixed with an addition of raw sulfid ore to bring the sulfur contents up to 10% gives a very satisfactory desulfurization and sintering in 115 the blast roaster.

The sintered mass is then broken into com- 120 paratively coarse lumps such for example as will pass through a half inch screen the coarseness of the grain being to some extent determined by the character of the sinter. This roasted or desulfurized product in the form of relatively coarse and porous pieces is then mixed with coal and charged into the distillation retorts in the 125 ordinary way when the reduction takes place with ease and rapidity it being found that a reduced amount of fuel is necessary for the reduction while the retort yield is increased and in all respects the advantages 130

are obtained which would be expected to accrue from the use of a coarsely divided ore being at the same time sufficiently porous for the passage of the reducing gases.

5 It has been found desirable to use a binding material to prevent the charges on the grate of the blast roaster forming blow holes and to reduce dust losses carried over mechanically with the air blast. I have 10 found zinc blende in the form of slime concentrates effective in overcoming these difficulties. These slime concentrates are in a very finely divided condition and when mixed with water form a more or less plastic 15 mass which acts as a most effective binder for the sulfids on the grates of the blast roaster besides providing the necessary amount of green sulfids for admixture with the pre-roasted ore. By damping the 20 pre-roasted ore with a mixture of water and these slime concentrates and then subjecting the same to ignition and blast roasting the difficulty of blow holes can be overcome and the dust losses reduced to a minimum. When slimes are not available 25 plastic clay may be used in the same way with good results.

The temperature resulting from the combustion of the sulfur may be further controlled in the blast roaster by mixing with the air or atmosphere being drawn or forced through the ignited body of ore a certain proportion of steam or water vapor. The proportion of steam to the air or oxidizing atmosphere is determined according to the amount necessary to avoid the generation of heat sufficient to fuse and slag the particles.

When it is desirable to utilize sulfur dioxide gases obtained by the desulfurizing or roasting of the ores for the purpose of manufacture of sulfuric acid it may be found that by this method of treatment the gases coming from the final roast or desulfurization on the blast roaster are not sufficiently rich in sulfur dioxide for economical manufacture of acid. In such cases the aforesaid gases may be enriched by drawing the gases or a portion of the gases from 45 the blast roaster and passing them over one or more hearths of the preliminary roasting furnace. In this way the gases may be enriched as to their sulfur dioxide contents and thereby be of sufficient strength 50 for manufacture of sulfuric acid.

In practice it is found that ore treated in this way may be desulfurized to such an extent as is necessary for all practical purposes and that the resultant sintered mass 55 is in a fine porous condition which may be easily broken and is found to be in a very suitable condition for treatment in retorts for distillation of spelter or for leaching preparatory to electro-deposition or the production of zinc oxid.

1 claim—

1. In the art of roasting zinc sulfid ores the process which consists in subjecting the ore to a preliminary roast and then subjecting to a blast roast, the preliminary roast 70 eliminating sulfur to such a degree that the blast roast produces a porous sinter.

2. The desulfurizing of zinc sulfid ores (blende) characterized by the production of a roasted product in coarse grained form 75 and intimately porous in which form it is peculiarly suited to treatment in the distillation process, said desulfurizing being effected in two separate operations, which comprise first subjecting the ore to a preparatory roasting for the dilution of the sulfur contents to such an extent that fusion and slagging are avoided in the subsequent blast roasting operation, the said preparatory roasting leaving the ore in a fine granular 85 condition, and then blast-roasting the said ore for the further elimination of sulfur and until a sintered product is formed of a relatively coarse and porous character the porosity of the sintered product thus obtained 90 being sufficient for the free passage of the gases generated in zinc distillation retorts.

3. In the desulfurizing of zinc sulfid ores first subjecting the ore to a partial roast for the dilution of the sulfur contents then mixing such partially roasted ore with green or unroasted zinc sulfids in proportions that the sulfur contents of the mixture are such that fusion and slagging are avoided in the subsequent operation and subjecting the mixture 100 to a blast roasting operation for the elimination of the sulfur and the formation of a sintered product.

4. In the desulfurizing of zinc sulfid ores subjecting the ore to a more or less complete 105 roast (such as a dead roast) mixing such roasted ore with green or unroasted zinc sulfids in proportions that the sulfur contents of the mixture are such that fusion and slagging are avoided in the subsequent operation and then subjecting the mixture to a blast roasting operation for the elimination of the sulfur and the formation of a sintered product substantially as described.

5. In the desulfurizing of zinc sulfid ores 115 first subjecting the ore to a partial roast then mixing such partially roasted ores with water containing green zinc sulfid slimes in proportion that the sulfur contents of the mixture are such that fusion is avoided in the 120 subsequent operation subjecting the mixture to a blast roasting operation for the elimination of the sulfur and the formation of a sintered product substantially as described.

6. In the desulfurizing of zinc sulfid ores 125 first subjecting the ore to a partial roast then mixing such partially roasted ore with a certain proportion of green sulfids moistening the mixture with a binding agent and subjecting the mixture to a blast roasting oper- 130

ation for the elimination of the sulfur and the formation of a sintered product substantially as described.

7. In the desulfurizing of zinc sulfid ores 5 first subjecting the ore to a partial roast, said partial roast leaving it in a fine grained condition, adding a binding agent to the partially roasted ore said binding agent being of a character which will be effective below 10 the sintering temperature of the charge to prevent the finely-divided particles from running through the grate of the subsequently employed blast roaster or from thereafter forming blow holes thereon, and 15 finally subjecting the charge to a blast roasting operation for the further elimination of sulfur and the formation of a sintered product of a relatively coarse and porous character; substantially as described.
- 20 8. In the desulfurizing of zinc sulfid ores first subjecting the ore to a partial roast then mixing such partially roasted ores with a certain proportion of green or unroasted zinc sulfids, moistening the mixture with 25 water containing green or unroasted zinc sulfid slimes and subjecting the mixture to a blast roasting operation for the elimination of the sulfur and the formation of a sintered product substantially as described.

9. In the desulfurizing of zinc sulfid ores 30 first subjecting the ore to a partial roast then mixing such partially roasted ores with a certain proportion of green or unroasted zinc sulfids, moistening the mixture with water containing clay and subjecting the mixture 35 to a blast roasting operation for the elimination of the sulfur and the formation of a sintered product substantially as described.

10. In the desulfurizing of zinc sulfid ores (blende) first partially roasting the ore for 40 the dilution of the sulfur contents then mixing such partially roasted ore with green or unroasted zinc sulfids and then subjecting the mixture to a blast roasting operation introducing steam or water vapor with the air 45 being drawn or forced through the ignited body of ore in such proportions as may be necessary to avoid fusing and slagging whereby the elimination of the sulfur is effected with the formation of a sintered product substantially as described.

In testimony whereof I have affixed my signature in presence of two witnesses.

GILBERT RIGG.

Witnesses:

ANNA HACK,  
G. R. CULLEN.